

1

3,594,156  
STAINLESS STEEL

Henry P. Leckie, Griffith, Ind., and Eugene Williams, Pittsburgh, Pa., assignors to United States Steel Corporation

No Drawing. Filed May 29, 1969, Ser. No. 829,110  
Int. Cl. C22c 37/10

U.S. Cl. 75—124

2 Claims

## ABSTRACT OF THE DISCLOSURE

A low cost ferritic stainless steel with exceptionally good corrosion resistant properties having the following composition:

|            |                |
|------------|----------------|
| Carbon     | 0.03% maximum. |
| Manganese  | 2.0% maximum.  |
| Chromium   | 6 to 12%.      |
| Aluminum   | 2 to 7%.       |
| Copper     | 0.1 to 1.5%.   |
| Molybdenum | 0.2 to 3.0%.   |
| Columbium  | 0.2 to 3.0%.   |
| Iron       | Balance.       |

wherein chromium plus aluminum is at least 13.0%, molybdenum plus columbium is at least 0.8% and copper plus molybdenum plus columbium is at least 1.0%.

## BACKGROUND OF THE INVENTION

This invention relates generally to stainless steel, and more specifically, to a new, low cost, 6 to 12 percent chromium stainless steel having corrosion resistance equal to or better than the conventional 18 percent chromium stainless steels.

The superior corrosion resistance of commercial stainless steels is primarily due to the addition of chromium to the alloy in amounts which vary from 4 to 30%. Since the corrosion resistance of stainless steel is more or less a direct function of the chromium content, it is well accepted that those stainless steels having large amounts of chromium are usually superior in corrosion resistance to those having lesser amounts.

The three most common stainless steels in commercial use today are the AISI (American Iron and Steel Institute) Types 410, 430 and 304 which contain about 12, 17 and 18% chromium respectively. Of these three most common stainless steels, AISI Type 304, having the greatest amount of chromium, is the best for conventional corrosion resistance applications.

In addition to being the primary constituent for corrosion resistance, chromium is also the principal cost element in commercial stainless steels. Therefore, AISI Type 304 stainless steel, in addition to being superior in corrosion resistance, is also more expensive than AISI Types 410 and 430 or most other lower chromium stainless steel.

Because of the relatively high cost of chromium, there are continuing efforts to find replacements for at least a portion of chromium by other cheaper elements that would reduce production costs yet maintain a reasonably high degree of corrosion resistance.

## SUMMARY OF THE INVENTION

This invention is predicated upon our development of a new stainless steel wherein a portion of the chromium content is replaced by controlled amounts of aluminum, copper, molybdenum and columbium. This lower cost stainless steel contains chromium in amounts of from 6 to 12 percent, and yet has corrosion resistance characteristics equal to or greater than AISI Type 304 stainless steel.

2

Accordingly, it is an object of this invention to provide a new low cost stainless having exceptionally good corrosion resistance and containing from 6 to 12 percent chromium and lesser controlled amounts of aluminum, copper, molybdenum, and columbium.

It is another object of this invention to provide a new low cost stainless steel having from 6 to 12 percent chromium and yet having corrosion resistance characteristics equal to or greater than the 18 percent chromium stainless steels.

It is a further object of this invention to provide a new stainless steel having corrosion resistance characteristics equal to or greater than AISI Type 304 stainless steel and yet utilizing lesser amounts of chromium.

## DESCRIPTION OF THE PREFERRED EMBODIMENTS

Although aluminum, molybdenum, columbium and copper are known to impart some small degree of corrosion resistance to steel, we have found that there are substantial beneficial interactions between certain combinations of these elements which even further contribute to corrosion resistance. Even relatively small combined amounts of chromium and aluminum; molybdenum and columbium; or copper, molybdenum and columbium will render exceptional corrosion resistant characteristics to a steel. We have further found that a combination of all three beneficial interactions can be used as a substitute for a large portion of the chromium in stainless steels without an adverse affect on corrosion resistance. These substituted elements being cheaper in cost, and/or being used in comparatively smaller amounts have the effects of making a high quality stainless steel cheaper to produce and yet maintaining exceptional corrosion resistance characteristics. A stainless steel in accordance with this invention therefore may have corrosion resistance characteristics equal to or better than AISI Type 304 stainless steel while containing about half, or even less than half as much chromium and low cost quantities of aluminum, copper, molybdenum and columbium.

The stainless steel of this invention has the following general composition:

|            |               |
|------------|---------------|
| Carbon     | 0.3% maximum. |
| Manganese  | 2.0% maximum. |
| Chromium   | 6 to 12%.     |
| Aluminum   | 2 to 7%.      |
| Copper     | 0.1 to 1.5%.  |
| Molybdenum | 0.2 to 3.0%.  |
| Columbium  | 0.2 to 3.0%.  |

The balance of the steel should of course be iron (i.e. iron with other usual steel making impurities). Chromium and the chromium substituted elements must be present in the following minimum combined amounts:

|                                       |                   |
|---------------------------------------|-------------------|
| Chromium plus aluminum                | 13% minimum.      |
| Molybdenum plus columbium             | 0.8% minimum.     |
| Molybdenum plus columbium plus copper | per 1.0% minimum. |

Although as little as 2% aluminum will be beneficial to the corrosion resistant properties, optimum results are obtained only if aluminum is maintained within a range of 3 to 7% at an ideal chromium content of about 8%. In a like manner, copper, although beneficial at concentrations as low as 0.1%, is ideally maintained at about 1%. Chromium contents towards the higher end of the range will of course provide slightly better corrosion resistance. For most applications however, about 8% chromium, or from 6 to 10% is preferred as a practical good balance between corrosion resistance and economy. The beneficial effects of molybdenum and columbium

are somewhat proportional to their combined concentration up to a preferred concentration of about 1% each. Increasing the molybdenum and/or columbium content above the preferred 1% and 0.5% respectively will provide only slight improvements in corrosion resistance up to about 3% each. Beyond 3% of either element, no significant improvement is obtained.

Accordingly, the preferred composition of this stainless steel, for optimum corrosion resistance at a minimum cost, would be about 8% chromium, 3-7% aluminum and 1% each of copper and molybdenum and 0.5% columbium.

The effect of copper on corrosion resistance properties is actually detrimental at chromium contents below 6%,

comparing them with those values for commercially available stainless steels, the passivation tendency, and hence the corrosion resistance characteristics, for any experimental heat can be readily evaluated. A strong tendency to passivate is manifested by an active passivation potential and a low critical current density.

Table I below contrasts the critical current density and chemistry of AISI Type 430 stainless steel and twelve experimental heats, most of which have compositions in accordance with this invention. AISI Type 430 stainless steel is shown to have a critical current density of 7.2 ma./cm.<sup>2</sup>, while all experimental heats had critical current densities below that amount, and hence are superior in corrosion resistance.

TABLE I

| Example Number | Chemical composition, percent by weight |      |       |       |       |       |       |       |      |      |       |       |       | Critical current ma./cm. <sup>2</sup> |
|----------------|-----------------------------------------|------|-------|-------|-------|-------|-------|-------|------|------|-------|-------|-------|---------------------------------------|
|                | C                                       | Mn   | P     | S     | Si    | Ni    | Ti    | N     | Cr   | Al   | Cu    | Mo    | Cb    |                                       |
| AISI 430.....  | 0.07                                    | 0.65 | 0.02  | 0.007 | 0.52  | 0.39  | 0.05  | 0.08  | 17.1 | 0.01 | 0.05  | 0.05  | ----- | 7.2                                   |
| 1.....         | 0.02                                    | 0.51 | 0.02  | 0.017 | 0.96  | 1.04  | 0.11  | 0.01  | 5.01 | 7.10 | 0.11  | 0.57  | 0.04  | 6.6                                   |
| 2.....         | 0.02                                    | 0.55 | 0.02  | 0.018 | 1.06  | 0.20  | 0.50  | 0.01  | 8.72 | 2.78 | 0.09  | 0.55  | 0.49  | 7.0                                   |
| 3.....         | 0.02                                    | 0.46 | 0.03  | 0.018 | 0.5   | 1.13  | 0.29  | 0.01  | 6.32 | 4.75 | 0.50  | 1.00  | 0.28  | 2.7                                   |
| 4.....         | 0.02                                    | 0.55 | 0.03  | 0.019 | 0.5   | 0.18  | 0.32  | 0.01  | 7.03 | 5.51 | 0.50  | 0.80  | 0.28  | 3.1                                   |
| 5.....         | 0.02                                    | 0.52 | 0.03  | 0.021 | 0.5   | 2.31  | 0.28  | 0.01  | 6.64 | 4.49 | 0.52  | 0.79  | 0.30  | 3.6                                   |
| 6.....         | 0.02                                    | 0.55 | 0.03  | 0.016 | 0.5   | 0.62  | 0.32  | 0.01  | 7.00 | 5.34 | 0.50  | 0.79  | 0.28  | 3.3                                   |
| 7.....         | 0.014                                   | 0.53 | 0.006 | 0.010 | 0.11  | <0.01 | 0.51  | 0.008 | 8.50 | 4.78 | 0.052 | 0.58  | 0.52  | 5.7                                   |
| 8.....         | 0.025                                   | 0.50 | 0.005 | 0.006 | 0.028 | <0.01 | 0.29  | 0.006 | 8.00 | 4.98 | 1.05  | 0.55  | 0.12  | 4.25                                  |
| 9.....         | 0.015                                   | 0.61 | 0.007 | 0.007 | 0.023 | <0.01 | 0.30  | 0.008 | 8.33 | 4.67 | 1.04  | 0.21  | 0.49  | 3.6                                   |
| 10.....        | 0.005                                   | 0.50 | 0.007 | 0.004 | <0.03 | <0.01 | ----- | 0.011 | 8.66 | 3.87 | 1.04  | 1.02  | 0.69  | 3.3                                   |
| 11.....        | 0.003                                   | 0.51 | 0.005 | 0.005 | <0.03 | <0.01 | ----- | 0.010 | 8.65 | 5.22 | 0.75  | 0.03  | 0.69  | 3.0                                   |
| 12.....        | 0.006                                   | 0.52 | 0.005 | 0.003 | <0.03 | <0.01 | ----- | 0.010 | 8.47 | 4.93 | 1.03  | 0.018 | 0.037 | 5.5                                   |

but of course beneficial at chromium levels above 6%. Therefore, the minimum chromium content of 6% is critical to avoid the adverse affects of copper.

Nickel and silicon additions were considered for this alloy, but neither showed any beneficial effect. Nickel is neither beneficial nor detrimental. Silicon, on the other hand, not only has a detrimental effect on corrosion resistance, but further adversely affects the metallurgical quality of the steel. Therefore, silicon should be kept at residual impurity amounts of less than 1.0%.

In order to quantitatively evaluate the stainless steels of this invention, potentiodynamic polarization tests were performed. This test is based upon the fact that stainless steels achieve their high resistance to corrosion by their ability to spontaneously passivate (i.e. form a protective oxide film) in the corrosive environment. Although active metal such as iron can be made to passivate electrolytically by the application of an electrical current or potential in a proper solution, the "stainless" metals inherently passivate without the applied force. The driving force for the electrochemical reaction is provided by the currents resulting from local variations in potential at the metal surface. The inherent ability to form a protective film (passivate) requires that this reaction have a thermo-

In Table I above, it is readily apparent that the stainless steels having compositions in accordance with this invention do have substantially lower critical current densities than the AISI Type 430 stainless steel, and hence, substantially greater corrosion resistance tendencies. Of 35 the twelve experimental heats, only four show critical current densities of less than 2.0 m./cm.<sup>2</sup> lower than AISI Type 430, namely Examples 1, 2, 7 and 12. It should be noted that these four examples are the only ones not in accord with our composition requirements. (Note underlined figures outside our ranges.) Example 1 has an excessive amount of aluminum; Examples 2 and 7 an insufficient amount of copper; and Example 12 an insufficient amount of molybdenum and columbium. In addition, Example 2 further characterizes the adverse affect of silicon.

Table II below contrasts the critical current density and chemistry of AISI Type 304 stainless steel and five experimental heats according to a somewhat more preferred composition of this invention. Table II is substantially the 50 same as Table I above except that a better stainless steel (i.e. AISI Type 304) is used as the standard. Therefore the experimental heats compared thereto are within our preferred composition range.

TABLE II

| Example Number | Chemical composition, percent by weight |      |       |       |        |       |       |       |       |      |      |      |      | Critical current ma./cm. <sup>2</sup> |
|----------------|-----------------------------------------|------|-------|-------|--------|-------|-------|-------|-------|------|------|------|------|---------------------------------------|
|                | C                                       | Mn   | P     | S     | Si     | Ni    | Ti    | N     | Cr    | Al   | Cu   | Mo   | Cb   |                                       |
| AISI 304.....  | 0.02                                    | 0.60 | 0.02  | 0.018 | 1.00   | 1.00  | 0.48  | 0.02  | 9.17  | 6.13 | 1.04 | 1.04 | 0.59 | 2.8                                   |
| 1.....         | 0.016                                   | 0.53 | 0.005 | 0.009 | 0.12   | <0.01 | 0.49  | 0.009 | 8.38  | 5.18 | 1.10 | 1.04 | 0.53 | 1.2                                   |
| 2.....         | 0.006                                   | 0.50 | 0.005 | 0.003 | <0.003 | <0.01 | ----- | 0.011 | 8.90  | 5.06 | 1.06 | 1.05 | 0.70 | 2.4                                   |
| 3.....         | 0.007                                   | 0.50 | 0.006 | 0.004 | <0.03  | <0.01 | ----- | 0.009 | 8.84  | 4.80 | 1.07 | 1.05 | 0.50 | 1.9                                   |
| 4.....         | 0.004                                   | 0.51 | 0.005 | 0.009 | 0.02   | ----- | ----- | 0.02  | 10.00 | 4.13 | 1.07 | 0.66 | 0.40 | 2.5                                   |
| 5.....         | 0.006                                   | 0.53 | 0.005 | 0.009 | 0.02   | ----- | ----- | 0.02  | 12.10 | 4.18 | 1.09 | 0.68 | 0.41 | 1.5                                   |
| 6.....         | 0.007                                   | 0.52 | 0.005 | 0.006 | 0.02   | ----- | ----- | 0.02  | 11.00 | 4.18 | 1.06 | 0.67 | 0.41 | 2.0                                   |
| 7.....         | 0.005                                   | 0.54 | 0.006 | 0.008 | 0.04   | ----- | 0.48  | 0.04  | 9.17  | 6.13 | 1.04 | 0.53 | 0.48 | 1.7                                   |

dynamic and kinetic tendency greater than any other electrode reaction that might possibly take place.

A metal is passive if, on increasing the electrode potential towards more noble values the rate of anodic dissolution in a given environment under steady-state conditions becomes less than the rate at same less noble potential. The tendency for passivation of stainless steels is a function of both a critical current density and a critical potential. Therefore, by measuring these parameters and

70 75 From the two tables above it is apparent that AISI Type 304 stainless steel is indeed superior in corrosion resistance to AISI Type 430. Type 304 has a critical current value of 2.8 ma./cm.<sup>2</sup> whereas Type 430 has a critical current value of 7.2 ma./cm.<sup>2</sup>. This variation is of course well accepted.

In Table II above, it is readily apparent that the stainless steels having compositions in accordance with our preferred embodiment of this invention have lower critical

current densities than even the AISI Type 304 stainless steel, and hence comparable or better corrosion resistance tendencies.

The above potentiodynamic polarization tests were verified by exposing samples of our stainless steel along with samples of AISI Type 430 and 304 stainless steels, to the corrosive atmospheres of a coke making plant. After seven months exposure our stainless steels were substantially less corroded than the AISI Type 430 steels and exhibited corrosion resistance comparable to or better than the AISI Type 304 stainless steels.

We claim:

1. A low chromium ferritic stainless steel consisting essentially of up to 0.03% carbon, up to 2.0% manganese, 6 to 12% chromium, 2 to 7% aluminum, 0.1 to 1.5% copper, 0.2 to 3.0% molybdenum, 0.2 to 3.0% columbium and the balance substantially iron, the chromium, aluminum, copper, molybdenum and columbium being present in the following combined minimum amounts:

|                                       | Percent |
|---------------------------------------|---------|
| Chromium plus aluminum                | 13      |
| Molybdenum plus columbium             | 0.8     |
| Molybdenum plus columbium plus copper | 1.0     |

5 2. A low chromium stainless steel according to claim 1 having about 8% chromium, 3-7% aluminum, and about 1% each of copper, molybdenum, and columbium.

#### References Cited

##### UNITED STATES PATENTS

|           |         |         |        |
|-----------|---------|---------|--------|
| 2,848,323 | 8/1958  | Harris  | 75—124 |
| 3,288,600 | 11/1966 | Johnsen | 75—125 |

10 15 HYLAND BIZOT, Primary Examiner

U.S. Cl. X.R.

75—125, 126C, 126F